

## UNITED STATES PATENT OFFICE

2,633,730

## PROCESS OF FINISHING FISH SKINS

Henry Rose, Gloversville, N. Y.

No Drawing. Application February 2, 1951,  
Serial No. 209,211

3 Claims. (Cl. 69—21)

1

This invention relates to a process of preparing fish skins employing a combined tanning and burning operation whereby the skins secure a unique, smooth, and uniformly attractive appearance, and the skins are rendered serviceable for a multitude of uses.

An important object of this invention is to provide a process of preparing attractive and serviceable fish skins of unique uniform appearance, which process can be carried out easily and efficiently.

A further object of this invention is to provide a process of the character described wherein, by combining a tanning and burning operation, together with a color or dyeing operation and a glazing operation, a smooth, serviceable and uniform product results having a novel two-tone effect. The process can be effectively employed for the preparation and treatment of the skins of such fish as salmon, Atlantic salmon, steel-head trout, trout species, herring species, halibut, flounder species, cod species, rock fish species, tuna species, and the like.

The present process will be described immediately hereinafter and it will be evident to those skilled in the art that several of the operations included in the process are conventionally employed for the conversion of fish skins to leather. The skins are soaked in water overnight and washed out salt-free with water at room temperature, or approximately 70° F., after which the skins are fleshed, either manually or mechanically, and again washed for approximately fifteen minutes with water maintained at a temperature of approximately 45–75° F. Thereafter, the skins are subjected to a swelling operation which removes most of the scales. Any alkali, such as sodium or potassium hydroxide, or lime, or sodium sulphide, can be employed, alone or in various combinations, in a solution containing 0.5 to 1.0% by weight of the alkali, the skins remaining in this solution from one to three days, it being preferred that the alkali be present in an amount of 2.0 to 10.0% by weight of the skins treated. Thereafter, the skins are washed thoroughly for two to three hours until the swelling is completely removed. The above-described soaking, fleshing, and swelling operation is conventional in the art.

Inasmuch as these operations fail to completely remove the scales from the skin, the skins are brushed or otherwise mechanically or manually treated to remove the remainder of the scales. After the complete removal of the scales from the skins, the skins are again washed with water

2

and subjected to bathing in the presence of pancreatic enzyme. Depending upon the kind of leather desired, the bathing can be carried on from one to twelve hours, the longer the treatment, the softer the leather. An aqueous solution of the pancreatic enzyme is employed in concentrations of 0.25 to 0.50% by weight, the temperature of the solution being maintained at approximately 45 to 70° F. and at a pH of 8.5 to 9.0.

10 The conventional procedure in the treatment of the fish skins after bathing is to split the skin with some of the scales thereon, but it has been found that such splitting causes unevenness in the structure of the skin, is very difficult to control, and results in the loss of a large percentage of the leather. The present process has been provided to overcome disadvantages of the splitting operation as will appear hereinafter.

15 After the bathing operation, the skins are again washed with water and are subjected to a tanning operation. The tanning is carried out in the presence of aqueous vegetable extracts, such as an extract of the quebracho bark or the extract of the sumac leaves, or may be carried out in 20 the presence of a synthetic material such as syntan, a condensation product of coal derivatives, such as a condensation product of naphthalene sulfonic acid and formaldehyde. The skins are maintained in the extracts for approximately two 25 to three days or until complete penetration takes place, the extract being employed in an amount ranging from 10 to 70% on the basis of the drain weight of the skins. It is preferred that the skins be maintained in the extract on the 10% level first, the extract increasing every two hours until 30 35 60 to 70% has been added.

At this stage, before vegetable tanning, the skins can be bleached, if desired, in the following way. The skins are immersed in an aqueous 40 solution of potassium permanganate for one-half hour or until the skins have a uniform reddish color. Potassium permanganate is employed in an amount equivalent to 0.25 to 1.0% by weight of the drained skins. After the skins are washed 45 and rinsed to remove the excess permanganate, they are treated with an aqueous solution of bisulphite, such as sodium or potassium bisulphite, or any other water soluble bisulphite, until the skins are substantially white and all pigmentation has disappeared. The bisulphite is employed 50 in concentrations equivalent to 2.0 to 3.0% by weight of the drained fish skins. After the bleached skins have been washed free of bisulphite, they are subjected to the vegetable tanning 55 described immediately hereinabove. It

should be remembered that various kinds of bleaching agents may be employed instead of the bisulphites, such as the peroxides in the presence of ammonia.

The bleaching operation can be carried out in still another manner. The skins may be run into a solution of 10° Bé. sodium chloride and 1.0 to 2.0% sulphuric acid on the basis of the drain weight of the skins. Thereafter 1.0 to 3.0% by weight of potassium permanganate is added and after approximately one-half hour 2.0 to 3.0% by weight of the bisulphite is added until the skins are completely bleached. The skins are then drained and a 6° Bé. salt solution is added in sufficient quantities to cover the skins. This bleaching operation can be immediately followed with a vegetable tanning operation in which a 20.0 to 30.0% by weight of quebracho or other vegetable extract may be added to the salt solution and the skins maintained in this combined salt and vegetable extract solution for approximately one hour, after which another 20.0% by weight of the extract is added and the skins are left in this solution until complete penetration of the skin occurs. After the penetration, the skins are washed out salt-free and are then ready for the fat-liquoring process.

If desired, the tanning of the fish skins may be carried out after the pickling and bleaching operation by a process conventionally known as chrome tanning. In this process, the skins, after pickling, are subjected to an aqueous solution of chromium sulphate employed in an amount approximately of 10.0% by weight of the drained skins. After two hours of treatment with the chromium sulphate, sodium bicarbonate is added until the pH is 4.6 and the skins are left to soak overnight. They should stand the boil test of 180-190° F. and are washed out at approximately 100° F. for approximately one-half hour and neutralized with sodium bicarbonate until the pH is 5.5. The skins are then treated with 10% by weight of a vegetable extract, such as quebracho or sumac, after which the skins are ready for fat-liquoring. Any combination of known tannages may be applied for fish skins, like formaldehyde or formaldehyde and chrome combinations, and the like.

After the skins are vegetable-tanned as in any of the above processes, they are fat-liquored with 2.0 to 4.0% by weight of sulphonated cod oil (medium sulphonation), at a temperature of approximately 110 to 120° F. for approximately forty-five minutes. The skins are then hung up to dry and if they are crusted, after drying, they may be resoaked. After fat-liquoring the skins, they can be colored with any suitable dye such as 1.0% by weight of Acid Anthracene Red GA Ex. Conc. and Brilliant Croceine 3 BA at a temperature of approximately 100° F. The dyestuff is exhausted with a 0.5% formic acid and pasted. After the skins are pasted and dried out, they are staked and buffed on the flesh side.

At this stage, the skins are subjected to a burning or singeing operation which constitutes the heart of the present invention. This operation, in effect, burns off the tips of the scale pockets without burning or otherwise affecting the remainder of the skin so that a smooth and uniform fish skin results which has a unique and exceptionally attractive appearance. The pockets in which the scales are embedded are quite uniform in character, but they have a very thin layer of kollagen at the end of the pocket, which makes the appearance non-uniform.

During the process, the ends of the pockets become muggy and partly decomposed. Since, as pointed out hereinabove, splitting or any other operation like buffing produces non-uniform effects, the present burning or high temperature treatment produces the uniformity and attractive appearance desired and also improves the serviceability of the skins. The skins may be subjected to high temperatures, in the order of 800° C., using an electric plate, rollers, or a gas flame. The preferred operation is carried out by having a hot flame close to the surface of the skin, the skins being folded on a pipe thru which cold water is flowing, so that the high temperature of the flame will affect only the tips of the scale pockets and will not scorch the skins. Before the burning operation, it is advisable to brush the skin against the scales so that the pockets will stand out, it being understood that the burning will be more easily accomplished in some species of this skin, in which case the brushing will be unnecessary. Although the temperature of the burning or singeing is approximately 800° C., it should be understood that heavier skins can tolerate more burning at somewhat higher temperatures, whereas the lighter skins will have to be adjusted accordingly. Electric rollers may be employed instead of a direct flame and both means may be employed to obtain different effects on the product. This burning operation can also be applied to any reptile skins, like snakes, e. g., boas, pythons, etc., in a similar manner.

And finally, the skins are brushed, glazed and plated, preferably under a Sheridan plating machine at a temperature of approximately 200° F. The brushing and glazing may be repeated as desired and after the glazing, it will be seen that a very attractive two-tone effect is obtained. In the event that the skins are not colored after the vegetable tanning process, the skins can be table-colored, using acid or basic dyes, by swabbing the colors on the skins, and after the skins are dry they can be subjected to the burning or singeing operation described immediately hereinabove. After the vegetable or chrome tanning, if desired, the skins can be shaved on a shaving machine, in which case the staking and buffing may be omitted. It will also be understood that a machine arrangement can be employed for the singeing or burning and brushing operation as well as a hand-operated blow torch.

The following examples will illustrate several ways in which the present process has been carried out.

#### Example 1

One hundred fish skins were soaked in water at room temperature of approximately 70° overnight, and on the second day washed salt-free with water at a temperature of 45 to 70° F. and then fleshed. The skins were subjected to a swelling operation to remove a portion of the scales by washing at 45 to 70° F. for one-half hour in a solution containing 50 gallons of water and 2.50 lbs. of soda ash, and the skins were allowed to remain in this alkali solution overnight. The skins were then washed for approximately one-half hour with water at a temperature of approximately 80° F. and then subjected to the bathing operation employing 50 gallons of water and 2.0 lbs. of Oropon A. The bathing is followed with a tanning operation in which the skins are first washed with water at approximately 70° F. for one-half hour and

then soaked in a solution for one-half hour containing 25 gallons of water, 2.0 lbs. sumac, and 1.0 lb. syntan. 2.0 lbs. more of sumac is added within an hour and the skins are left to soak overnight. On the next day, another 2.0 lbs. of sumac is added over a period of two hours and the skins are allowed to soak overnight. The skins are then shaved and washed for one-half hour with water at approximately 120° F. and then washed for one-half hour with a 10 detergent solution at approximately 120° F. containing 10 gallons of water and 1.0 lb. sulphonated cod oil. The skins are then pasted, staked, buffed, burned or singed, brushed, glazed and plated in the manner described hereinabove.

*Example II*

In this example, 100 fish skins are treated to a soaking, fleshing and bating operation in a manner which differs from that described in Example I. However, the tanning, singeing and other operations as described in Example I remain the same. The fish skins are washed with water salt-free and are fleshed and washed cold at a temperature of 45 to 70° F. in ten minutes. The skins are then immersed in an aqueous solution of sodium sulphide in an amount of 2.0% by weight of the fish skins. The skins are then washed with water at a temperature of approximately 70° F. and then subjected to a solution for one-half hour of 20 gallons of water and 0.5 lbs. of sodium bicarbonate. The skins are again washed with water and unscaled either by hand or by machine and then again washed with water for twenty minutes at a temperature of approxi- 35

5 mately 80° F. The skins are then bated for two hours in a solution containing twenty gallons of water and 1.0 lb. Oropon A. After appropriate washing of the bated skins, they are tanned and otherwise treated as set forth in Example I.

6 While a preferred embodiment of the invention has been described hereinabove, it will be understood that minor variations may be made in the process without departing from the spirit of the invention and the scope of the appended claims.

Having described the process, what is claimed as new is:

1. A process for treating a fleshed, descaled, bated, tanned and fat liquored fish skin which consists of the step of burning off the tips of the scale pockets without burning the remainder of the skin.
2. The process of claim 1 wherein the burning is carried out at approximately 800° C.
3. The process of claim 1 and the step of glazing and plating the skin after the burning operation.

HENRY ROSE.

25 REFERENCES CITED

The following references are of record in the file of this patent:

30 UNITED STATES PATENTS

| Number    | Name      | Date          |
|-----------|-----------|---------------|
| 1,230,266 | Bendixen  | June 19, 1917 |
| 2,181,243 | MacDonald | Nov. 28, 1939 |
| 2,222,656 | Erkel     | Nov. 26, 1940 |
| 2,272,935 | Cotton    | Feb. 10, 1942 |